# EUROPEAN PATENT SPECIFICATION

(11) **EP 0 012 020 B1**
(45) Date of publication and mention of the grant of the patent: **26.01.1983**
(21) Application number: 79302730.1
(22) Date of filing: 29.11.1979
(51) Int. Cl.: G03C 1/84, G03C 1/02, C09B 23/00

(54) **Dry silver photo-sensitive compositions, dyes for use therein and preparation of such dyes**
Durch Wärme entwickelbare lichtempfindliche Silbersalzmaterialien, Farbstoffe hierfür und Herstellung dieser Farbstoffe
Compositions photosensibles aux sels d'argent développables à chaud, colorants pour celles-ci et préparation de ces colorants

(30) Priority: 29.11.1978 GB 4645978; 29.11.1978 US 964479; 29.11.1978 US 964480
(43) Date of publication of application: 11.06.1980
(73) Proprietor: MINNESOTA MINING AND MANUFACTURING COMPANY, St. Paul, Minnesota 55101 (US)
(72) Inventor: Lea, Bernard Alan, Pinnacles Harlow, Essex (GB); Burrows, Ronald William, Pinnacles Harlow, Essex (GB); Reece, Jack E., Saint Paul, Minnesota 55101 (US); Brown, Harvey A., Saint Paul, Minnesota 55101 (US)
(74) Representative: Baldock, Hugh Charles

## Description

This invention relates to compounds suitable for use as acutance dyes in photosensitive compositions, to the preparation of such compounds and to photosensitive compositions containing the compounds. The invention is particularly concerned with photosensitive compositions of the type known as "dry silver" compositions.

Dry silver photosensitive compositions comprise an intimate mixture of a light sensitive silver halide and another silver compound such as a silver salt of an organic acid, e.g. silver behenate or silver saccharine, which upon reduction gives a visible change and which is substantially light-insensitive. Such a mixture is usually prepared in suspension and the resulting dispersion spread as a layer on a suitable substrate. When dry, the layer is exposed to a light image and thereafter a reproduction of the image can be developed by heating the layer in the presence of a reducing agent such as hydroquinone or certain substituted phenols.

It is because the exposure and development of the layer occur without using water, that these materials are often referred to as dry silver light-sensitive materials. Such materials in which minor amounts of a photosensitive silver halide catalyst-progenitor are associated in catalytic proximity with major amounts of a heat sensitive oxidation-reduction image forming reaction mixture which reacts more rapidly in the presence of the catalyst resulting upon exposure of the silver halide are well known in the art. Examples of such materials are described in our British Patent No. 1 110 046 and in United States Patent Specification Nos. 3 839 049 and 3 457 075.

We believe, that when the mixture is exposed to light, a latent image is formed in the silver halide. Thereafter, the silver compound can be reduced by heating with the reducing agent, this reduction being catalysed image-wise by the light exposed silver halide. By a suitable choice of temperature, the reduction of the silver compound can be catalysed in the light exposed areas to give a visible darkening while any slight reduction which occurs in the non-light exposed areas is insufficient to give a marked change. Of course, because the silver halide acts as a catalyst progenitor, only very small amounts of it can suffice, e.g. 0.1 to 10% by weight of the mixture. However, large amounts, e.g. up to 15 or even 20% may be desirable in some circumstances.

In order to improve the sharpness or definition of photographic images a dye known as an acutance dye is often incorporated into photosensitive compositions. To be effective the acutance dye will absorb at the wavelengths at which the photosensitive composition is sensitive. The longer the path length of the light in the layer of light sensitive composition the greater the attenuation. Therefore, scattered light is attenuated or absorbed to a larger extent than light which impinges directly on a light-sensitive crystal. As a result therefore, although the overall speed of the composition is reduced slightly, scattered light and other light rays which are liable to produce a blurred image are preferentially absorbed and so the overall definition and sharpness of images produced in the layer are increased.

An acutance dye for use in a dry silver composition is preferably heat labile, that is to say, it is destroyed by the heat development of the dry silver composition to one or more compounds which are substantially colour-less.

United States Patent Specification Nos. 4 033 948, 3 984 248 and Reissue 29,168 disclose bleachable methine dyes which are photobleachabie or heatbleachable, the dyes are useful in photothermographic materials.

French Patent Specification No. 965 555 discloses a range of benzothiazole and benzoxazole cyanine dyes for use in conventional photographic emulsions and Chem. Ber. 101, 2925-30 (1968) discloses several compounds having a methine chain. There is no indication, in either of these references of the use of the compounds in photothermographic systems.

It is an object of this invention to provide dry silver compositions containing acutance dyes, which absorb light at at least some of those wavelengths to which the composition is sensitive and which are rendered colourless upon heat development of the dry silver composition.

It is also an object of the invention to provide novel compounds suitable for use as acutance dyes in dry silver systems and a method for their preparation.

According to the present invention there is provided a light-sensitive composition comprising an intimate mixture of a substantially light-insensitive silver compound which upon reduction gives a visible change and sufficient of a silver halide to catalyse said reduction to give a visible change in those areas where the silver halide has been exposed to light and when the mixture is heated in the presence of a reducing agent, the composition containing an acutance dye, characterised in that the acutance dye is a compound of the general formula: in which R¹ represents an alkyl group containing 1 to 12 carbon atoms,
R² represents a hydrogen atom, an alkyl group of 1 to 4 carbon atoms, a phenyl group, a substituted phenyl group of molecular weight less than 350, -COOR' in which R¹ is as defined above, C₆H₅CO― or R⁶NH.CO in which R⁶ represents a hydrogen atom or an alkyl, aryl or aralkyl group,
R³, R⁴ and R⁵ independently represent a hydrogen atom or a substituent which can be present in a cyanine dye type heterocyclic nucleus,
D represents in which R⁷ represents an alkyl group containing 1 to 4 carbon atoms,
Y represents -CN or ―NO₂,
n is 1 when k is 0 or k is 1 when n is 0, and
m is 0, 1 or 2,

the free bonds in the methine group of the acutance dye being satisfied by hydrogen or substituents conventional in such groups in methine dyes and those free bonds when D is being satisfied by hydrogen or substituents which can be present in a cyanine dye type heterocyclic nucleus.

The substituents R³, R⁴ and R⁵ independently represent a substituent which, as known in the art, can be present in a cyanine dye type heterocyclic nucleus, defined herein as a "cyanine dye compatible substituent", referring to the broadly art accepted knowledge of substituents. A range of such substituents are disclosed for example in United States Patent Specification No. 2 921 067.

Examples of substituents for R³, R⁴ and R⁵ include hydrogen or halogen, e.g. chlorine, bromine or iodine, an alkyl group containing 1 to 12 carbon atoms, an alkoxy group containing 1 to 4 carbon atoms, an alkenyl group containing 2 to 4 carbon atoms, -(CH₂)ₚCOOH where p is 0, 1,2 or 3, ―NO₂, -NH₂ or -NHCOCH₃, or any two of R³ to R⁵ together represent the carbon atoms needed to complete a fused on benzene ring. Preferably at least one, more preferably at least two, of the substituents R³ to R⁵ represent hydrogen atoms. The most preferred substituents to be represented by each of R³ to R⁵ are hydrogen, chlorine or bromine atoms, or methyl, ethyl, methoxy or ethoxy groups.

It is found that dry silver compositions containing one of the above described compounds as an acutance dye can give excellent sharp images and that the acutance dye will be rendered considerably lighter in colour or substantially colourless by the heating required to develop the composition. This is surprising in view of the fact that many of these dyes are found not to be decomposed to a colourless state when they are heated on their own to the temperature at which the dry silver compositions are heated for development.

The exact mechanism for this decomposition is not known although the extent of decolourisation has been found to vary when the dry silver systems are altered. Thus a dye may be decomposed to a colourless state when it is present in one particular dry silver system upon development but in a different system the dye may simply be rendered lighter in colour. Thus a compound for use as an acutance dye in a particular dry silver system is selected not only for its efficiency as an acutance dye in that system but also to obtain the desired background after the dry silver composition is developed.

One preferred group of acutance dyes for use in the invention are those in which k=0, n=1, Y is NO₂ and R² is COOC₂H₅, C₆H₅, C₁ to C₄ alkyl or hydrogen.

A second preferred group of acutance dyes for use in the invention are those in which m=1, k=1, n=0, Y is NO₂, D is oxygen or sulphur and R² Is COOR¹, C₆H₅, substituted phenyl, C₁ to C₄ alkyl-or hydrogen.

A further group of preferred dyes are 1-alkyl-4-nitromethylene-quinolanes in which the alkyl substituent contains 1 to 4 carbon atoms, particularly those dyes of the general formula (II): in which R¹¹ represents an alkyl group containing 1 to 4 carbon atoms, each R¹² independently represents a hydrogen or halogen atom, an alkyl or alkoxy group containing 1 to 4 carbon atoms, an alkenyl group containing 2 to 4 carbon atoms, ―(CH₂)ₚCOOH wherein p is 0, 1, 2 or 3, ―NO₂, ―NH₂ or NHCOCH₃, or two groups R¹² together represent the carbon atoms required to complete a fused on benzene ring. Preferably R" represents a methyl or ethyl group, at least one group R¹² represents a hydrogen atom and each other R¹² independently represents a hydrogen, chlorine or bromine atom, or a methyl, ethyl, methoxy or ethoxy group.

A further series of dyes are those of formula (I) in which R² represents: in which X, Z and Z' independently represent a hydrogen or halogen atom, NO₂, CN or perfluoroalkyl of 1 to 4 carbon atoms, with the proviso that at least one of X and Z is N0₂ and R³, R⁴ and R⁵ independently represent a hydrogen or halogen atom, an alkyl or alkoxy of 1 to 4 carbon atoms, alkenyl of 2 to 4 carbon atoms, ―(CH₂)_{P}COOH wherein p is 0, 1, 2 or 3, ―NO₂, -NH₂ or -NHCOCH₃, or any two of the adjacent groups are the atoms necessary to form a fused on benzene ring.

Preferred dyes within the group have the general formula (III): in which R'⁶ represents an alkyl group of 1 to 8 carbon atoms,
R¹⁷ represents alkyl or alkoxy of 1 to 8 carbon atoms, halogen, N0₂ or aryl, and
R₁₈ represents hydrogen, alkyl of 1 to 8 carbon atoms or alkoxy of 1 to 8 carbon atoms and X, Z and Z' have the meaning given, above.

The acutance dyes can be incorporated into the dry silver compositions of the invention in an amount from 5 x 10-⁴ to 0.1 mole of acutance dye per kilogram of total dry solids in the composition. Preferably, however the dyes are incorporated in an amount of from 2 x 10-³ to 3 x 10-² mole of acutance dye per kilogram of dry solids in the composition.

The light-sensitive compositions of the invention will normally be spread for use on a support, suitable supports including, for example, paper, polyester or polyamide film bases, and glass. The composition will normally be prepared as a solution or suspension which is spread as a layer on the support and then the solvent or vehicle is evaporated off to leave a dry photo-sensitive layer. If desired, a coating aid or binder such as polyvinyl butyral, polymethyl methacrylate, cellulose acetate, polyvinyl acetate, cellulose acetate-propionate and cellulose acetate butyrate, can be incorporated in the light-sensitive mixture.

The substantially light-insensitive silver compound is suitably a silver salt of an organic acid. The organic acid can be a C₁₂ to C₂₉ aliphatic acid and is preferably a C₁₆ to C₂₅ aliphatic acid. Examples include silver behenate, silver caprate, silver laurate, silver myristate, silver palmitate, silver stearate, silver arachidate and·silver saccharine.

The reducing agent for this substantially light-insensitive silver compound can normally be quite mild. Suitable examples include hydroquinone and substituted phenols such as 1-methyl-4-hydroxynaphthalene, methyl gallate, catechol, phenylene diamine, p-amino-phenol and 1-phenyl-3-pyrazolidone. The reducing agent can be incorporated into the light-sensitive composition. Alternatively, the composition can be placed in contact with the reducing agent after exposure to light. For example, a light-sensitive coating can be exposed to a light image, placed in contact with a layer containing the reducing agent and the image then developed by heating. Preferably, however, the reducing agent is incorporated in the light-sensitive composition before this is spread on the support. Then the storage stability of the composition can be improved by incorporating in the composition a small amount of a stabilizer such as an acid stabilizer, e.g. succinic acid, benzoic acid or salicylic acid.

The silver halide can be present in amounts of up to 20% by weight of the mixture of silver compounds or can be present in small amounts, e.g. 0.1 to 10% by weight of the mixture of silver compounds. It can be added as such to the substantially light-insensitive compound or formed in situ by adding a soluble halide, e.g. a mercury or sodium halide, to the substantially light-insensitive silver compound. The silver halide can, for example, be chloride, bromide or a mixture of them and/or other silver halides.

The light-sensitive compositions of the invention can include one or more sensitising dyes to improve their sensitivity to parts of the spectrum other than the shorter wavelengths. Thus dye sensitized dry silver compositions of the present invention can contain an additional acutance dye such as one of those described in our copending British Patent Nr. 1 565 593.

The compounds of general formula (I) may be prepared by a process which comprises reacting a compound of the general formula: wherein X⁹ represents an anion,
Z³ is selected from the group consisting of SR', wherein R' is as defined above, and with a compound of the formula: wherein Y and R² are as defined above, the reaction being conducted in the presence of a polar solvent, a base catalyst and an acid binding agent.

Suitable reagents are well known and fully exemplified in the cyanine/merocyanine dye literature.

The reaction is preferably carried out in the presence of C₂H₅OH as a solvent and (C₂H₅)₃N as both catalyst and acid binder. The preparation is analogous to known processes used in the synthesis of merocyanine dyes.

The acutance dyes of general formula (II) can be prepared by processes which are well known. Thus, they can be prepared in a manner analogous to the synthesis of simple merocyanine dyes as described, for example, in British Patent No. 426 718, by reacting nitromethane with a 1-alkyl-4-alkylthio-quinolinium salt in a solvent in the presence of a basic catalyst. They are, however, preferably prepared from 1-alkyl-quinolinium salts by the method described by Leonard, DeWalt and Leubuer in J.A.C.S., 73, 3328, in which a quinolinium quaternary salt is heated with nitromethane in the presence of a base, an oxidising agent and a solvent.

The dyes of general formula (III) may also be made according to the following reaction scheme A:

This method is performed in the presence of a strong tertiary amine such as diisopropylethylamine. For example, in forming 1,4-dihydro-4-(2,4-dinitrophenyl)-nitromethylene-1-methylquinoline (which may also be named 1,4-dihydro-1-methyl-4-(α,2,4-trinitrobenzylidene)-quinoline), one would react 4-nitromethylene-1-methyl-1,4-dihydroquinoline with 2,4-dinitrofluoro- benzenein diisopropylethylamine.

Certain of the compounds suitable for use as acutance dyes in the present invention are known. Certain compounds of the above formula in which m=0 are disclosed in J.A.C.S. 74, 2110, C.A. 55 27373g and United States Patent Specification No. 2 411 507 and other compounds in which m=1 are described by Severin & Bohme in Chem Ber. 101 2925-30 (1968). There is no indication in any of the prior art that such compounds would be suitable for use as acutance dyes in silver halide photothermographic emulsions.

Many of the compounds for use as acutance dyes in accordance with the invention are novel and therefore according to one embodiment of the invention there is provided a compound of the general formula: wherein:
R' represents an alkyl group containing 1 to 12 carbon atoms,
R³, R⁴ and R⁵ are cyanine dyes compatible substituents,
D represents a member of the group consisting of in which R⁷ is an alkyl group containing 1 to 4 carbon atoms,
n is 1 when k is 0 or k is 1 when n is 0,
m is 0, 1 or 2,

when m is 0 or 2:
R² represents an alkyl group of from 1 to 4 carbon atoms, a phenyl group, a substituted phenyl group of molecular weight less than 350, -COOR¹ wherein R¹ is as defined above, C₆H₈₅CO― or R⁶NH.CO- wherein R⁶ is a member of the group consisting of a hydrogen atom or an alkyl, aryl or aralkyl group,

and when m is 1:
R² represents R⁶NH.CO wherein R⁶ is as defined above, the free bonds in the methine group of the acutance dye being satisfied by hydrogen or substituents conventional in such groups in methine dyes and those free bonds when D is being satisfied by hydrogen or substituents which can be present in a cyanine dye type heterocyclic nucleus.

The invention will now be illustrated by the following Examples.

### Example 1

### Preparation of 4-(cyano-4'-nitrophenylmethylene)-1-methyl-quinolane (Compound No. 14)

1-Methyl-4-methylthio-quinolinium toluene-4-sulphonate (1.83 g) was placed in ethanol (20 ml) and 4-nitrophenylacetonitrile (0.81 g) added. The mixture was warmed, triethylamine (0.8 ml) added and the resulting mixture heated under reflux for 15 minutes. The dye which separated from the hot solution was filtered off and the crude compound (1.2 g) was twice crystallised from toluene (200 ml) to give magenta needles (0.9 g) having a melting point of 203 to 204°C. In methanolic solution the dye exhibited _{E} = ₂.₀ x 10° at A max 495 nm.

### Example 2

### Preparation of 4-(ethoxycarbonyl-nitromethylene)-1-methyl-quinolane (Compound No. 12)

1-Methyl-4-methylthio-quinolinium toluene-4-sulphonate (1.8 g) and ethyl nitroacetate (1 ml) were placed in ethanol (10 ml) and the mixture warmed. After the addition of triethylamine (0.7 ml) the whole was heated under reflux for 10 minutes. The product crystallised upon cooling and was filtered off. The crude product was purified by boiling with ethanol (70 ml), to give both an undissolved residue (0.8 g) and a crystallised sample (0.25 g). Both samples formed yellow plates with melting point of 203 to 206°C and the recrystallised sample showed ε = 6 x 10³ in methanolic solution at λ max 465 nm. Analvsis:

### Example 3

### Preparation of 3-ethyl-2(3-nitro-3-phenyl-allylidene)-2,3-dihydrobenzothiazole (Compound No. 21)

2-Acetanilino-3-ethyl-benzothiazolium iodide (4.5 g) was placed in ethanol (25 ml) and phenyl nitromethane (1.4 g) added. The mixture was warmed, triethylamine (1.4 ml) added and the resulting mixture heated under reflux for 20 minutes. Upon cooling, a mixture of product and trimethincyanine dye was deposited. This was filtered off and the product extracted with toluene. The extracted solid was then crystallised from ethanol (350 ml) to give dark green coloured plates (2.4 g) having a melting point of 155°C. In methanolic solution the dye exhibited ε=6.2 x 10⁴ at λ max 523 nm. Analysis:

### Example 4

### Preparation of 3-ethyl-2-(3-ethoxycarbonyl-3-nitro-allylidene)-2,3-dihydrobenzoxazole

### (Compound No. 20)

2-Acetanilino-3-ethyl-benzoxazolium iodide (2.17 g) was placed in ethanol (10 ml) and ethyl nitroacetate (1.0 ml) added. The mixture was warmed, triethylamine (0.7 ml) added and the resulting mixture heated under reflux for 7 minutes. The dye separated upon cooling and after filtration the crude product (1.2 g) was crystallised from toluene (17 ml) to give yellow needles (1.05 g) having a melting point of 172 to 175°C. In methanolic solution the dye exhibited ε=5.6 x 10⁴ at λ max 452 nm. Analysis:

### Example 5

### Preparation of 3-ethyl-2-(5-ethoxycarbonyl-5-nitro-penta 2,4-dienylidene)-2,3-dihydrobenzothiazole (Compound No. 34)

2-(4'-Acetanilino-1,3-butadienyl)-3-ethyl benzothiazolium iodide (4.76 g), ethyl nitroacetate (1.2 mi), ethanol (100 ml) and triethylamine were mixed and stirred at room temperature for 15 hours. The whole was then evaporated and the residue extracted with six portions (50 ml) each of toluene at 50°C. The residue obtained by evaporation of the toluene was crystallised from aqueous methanol to give dark microcrystals (0.5 g) with a melting point of 125°C. In methanolic solution the compound showed ε = 4.6 x 10⁴ at λ max 574 nm.

### Analysis:

### Example 6

### Evaluation of acutance dyes

A dry silver composition was first prepared. Under room light a 1000 g dispersion containing 12.5 parts of silver behenate in 87.5 parts of solvent which in turn comprised 75 parts butan-2-one and 25 parts toluene was charged to a mixing vessel maintained at 15°C. 20 g of polyvinyl butyral resin (commercially available from Monsanto under the trade mark Butvar, B-76) and 10 g of 1-methyl-2-pyrrolidinone were added and the mixture stirred for 30 minutes.

Under Wratten 1A safelight a mixture containing hydrobromic acid (15 ml, 2.0 molar in ethanol), hydroiodic acid (7 ml, 0.1 molar in ethanol), and mercuric bromide (4 ml, 0.5 molar in ethanol) was added with stirring. After 20 minutes an additional 40 g of Butvar B-76 was added, followed after five minutes by 10 g 2,6-bis-(2'-hydroxy-3-tertiary-butyl-5'-methyl-benzyl)-4-methyl-phenol available from American Cyanamide under the name A080 and 6 g phthalazinone. After 20 minutes 12 g of a solution containing 2 mg of the following dye: per gram of 1-methyl-2-pyrrolidinone was added and the mixture stirred for an additional 30 minutes.

Equimolar amounts of the acutance dyes to be tested were added to appropriate containers and dispersed in 2 ml of butane-2-one. 40 g portions of the light sensitive dispersion prepared above were added to each, the mixture shaken, left to stand 30 minutes, then shaken again prior to coating.

Knife coatings 100 µm thick on polyester sheets were prepared from each sample and dried 3.5 to 4.0 minutes at 90°C. These dried coatings were overcoated with a solution containing 97 parts butan-2-one and 3 parts vinyl chloride vinyl acetate copolymer available from Union Carbide under the name VYNS with the knife set 50 _{fl}m above the base and dried as before. The performance of these compositions was then evaluated.

A combination of a tungsten source, a narrow band filter at a wavelength closely matching the spectral absorbance of each dye and an aperture target overlaid with a 0 to 4 continuous density wedge in a vacuum frame, was used to make contact exposures at a wavelength closely matching the spectral absorbance maximum of each dye. The strips were then processed by heating for 20 seconds in a fluorochemical bath and examined for flare of the image.

The acutance property of the dyes was classified very good, fair by examining the sharpness of the image with the naked eye.

The background before and after processing was observed.

The following Table 1 reports compounds of the general formula (I) in which the free bonds are satisfied by hydrogen alone.

The mode of preparation of the compounds is indicated in the final column, in which:
1. refers to a preparation disclosed in Chem.Ber. 101 2295,
2. refers to a preparation analogous to Example 2,
3. refers to a preparation analogous to Example 3,
4. refers to a preparation analogous to Example 5.

### Example 7

A series of dyes of general formula (II) were prepared according to the method described in J.A.C.S. 73, 3328.

The dyes prepared are those having the values of R¹¹ and one of the substituents R¹², the remaining substituents R¹² representing hydrogen atoms, as set out in the following Table 2.

Compounds 36 to 43 were evaluated for use as acutance dyes in a similar manner to those in Example 6. Table 3 summarises the amount of each dye used in the dry silver compositions.

The acutance properties were measured as in Example 6 with the exception that microdensitometer traces across the width of the image at D = 2.0 (obtained after processing the exposed strips 20 seconds at 127°C in a fluorocarbon oil bath to give reproducible heating for these tests) were used to judge the effectiveness of each dye.

The widths reported are the measured widths in centimetres of the density profile of each image as obtained from the microdensitometer chart. All measurements were carried out at D = 1.5.

The results of testing the compositions are given in Table 4.

All exposures made at 480 nm.

As can be seen from these results the presence of a yellow acutance dye in a dry silver composition according to the invention significantly reduces flare as compared with the dry silver composition A not containing any acutance dye.

### Example 8

The following compounds of general formula (III) reported in Table 5 were prepared In accordance with reaction scheme (A).

In Table 5 the numbers in parentheses indicate the position of attachment for particular substituents. Infrared analysis and nucleus magnetic resonance analysis confirmed the structure of each of these dyes.

### Example 9

Four hundred grams of a dispersion containing 13 parts by weight of silver behenate in 87 parts of a solvent composed of 67 parts by weight methylethylketone, 26 parts by weight toluene, and 7 parts by weight methylisobutylketone was charged to a temperature-controlled stirred reaction vessel at 15°C. Dark room conditions were maintained during all subsequent work.

The following materials were added sequentially with 20 to 30 minutes of stirring between separate additions.
A. 2 g of 1-methyl-2-pyrrolidinone in 6 g of polyvinylbutyral,
B. 8 ml of 2M HBr (in ethanol) and 3.2 ml of 0.1 M HI (in ethanol),
C. 10 g of a copolymer derived from 91% by weight vinylchloride, 3% vinylacetate, and 6% by weight vinyl alcohol polymerized to a molecular weight of about 23,000, and 24 g of polyvinyl butyral,
D. 1.8 ml of 0.5M HgBr₂ (in ethanol) was added with 5 minutes of stirring,
E. 5.2 g of phthalazinone and 7.8 g of 2,6-bis-(2'-hydroxy-3'-t-butyl-5'-methylbenzyl)-4-methylphenol,
F. 2.8 ml of a sensitizer solution having 5 mg/ml of the sensitizer in N-methylpyrrolidone, the sensitizer having the formula:

10 mg of each candidate acutance dye was weighed into separate vessels with 3 ml of methylethylketone to dissolve or disperse the dye. 50 g portions of the light-sensitive dispersion formed above were combined with the dye solutions and to portions of methylethylketone alone as a control. All materials were stirred for three minutes. The portions were then allowed to stand at room temperature for 30 minutes, then they were knife coated at 85 pm thickness on polyester and dried for four minutes at 85°C. Each sample was top coated with a 50 pm knife coating of a vinylchloride/vinylacetate copolymer as a 5% by weight solution in methylethylketone.

The produced film samples were exposed at the wavelengths indicated below through a 0.25 mm aperture mask overlaid with a continuous density wedge in a vacuum frame. This permitted an easy comparison of image flare at equivalent optical densities after development for 15 seconds at 127°C in an inert fluorocarbon chemical bath. All dye samples had markedly less flare than the control samples, particularly at an optical density of 2.0. Except for the Compound No. 51, no samples left significant visible stain after processing. The dye of Compound No. 51 left a magenta stain which faded within an hour under room light. The dyes used in the tests were as follows:

### Compound No. 51 (560 nm),

### Compound No. 52 (500 nm),

## Claims

1. A light-sensitive composition comprising an intimate mixture of a substantially light-insensitive silver compound which upon reduction gives a visible change and sufficient of a silver halide to catalyse said reduction to give a visible change in those areas where the silver halide has been exposed to light and when the mixture is heated in the presence of a reducing agent, the composition containing an acutance dye, characterised in that the acutance dye is a compound of the general formula: in which R' represents an alkyl group containing 1 to 12 carbon atoms,
R² represents a hydrogen atom, an alkyl group of 1 to 4 carbon atoms, a phenyl group, a substituted phenyl group of molecular weight less than 350, -COOR' in which R' is as defined above, C₆H₅CO- or R⁶NH.CO in which R⁶ represents a hydrogen atom or an alkyl, aryl or aralkyl group,
R³, R⁴ and R⁵ independently represent a hydrogen atom or a substituent which can be present in a cyanine dye type heterocyclic nucleus,
D represents in which R⁷ represents an alkyl group containing 1 to 4 carbon atoms,
Y represents -CN or ―NO₂,
n is 1 when k is 0 or k is 1 when n is 0, and
m is 0, 1 or 2,
the free bonds in the methine group of the acutance dye being satisfied by hydrogen or substituents conventional in such groups in methine dyes and those free bonds when D is being satisfied by hydrogen or substituents which can be present in a cyanine dye type heterocyclic nucleus.

2. A composition as claimed in Claim 1 in which the acutance dye is a 1-alkyl-4-nitromethylene- quinolane, the alkyl substituent containing 1 to 4 carbon atoms.

3. A composition as claimed in Claim 2 in which the acutance dye has the general formula (II): in which R¹¹ represents an alkyl group containing 1 to 4 carbon atoms, each R¹² independently represents a hydrogen or halogen atom, an alkyl or alkoxy group containing 1 to 4 carbon atoms, an alkenyl group containing 2 to 4 carbon atoms, -(CH₂)ₚCOOH where p is 0, 1, 2 or 3, ―NO₂, -NH₂ or NHCOCH₃, or two groups R¹² together represent the carbon atoms required to complete a tused on benzene ring.

4. A light-sensitive composition as claimed in Claim 3 in which R" represents a methyl or ethyl group, at least one group R¹² represents a hydrogen atom and each other R¹² independently represents a hydrogen, chlorine or bromine atom, or a methyl, ethyl, methoxy or ethoxy group.

5. A composition as claimed in Claim 1 in which R² represents: in which X, Z and Z' independently represent a hydrogen or halogen atom, N0₂, CN or perfluoroalkyl of 1 to 4 carbon atoms, with the proviso that at least one of X and Z is N0₂ and R³, R⁴ and R⁵ independently represent a hydrogen or halogen atom, an alkyl or alkoxy of 1 to 4 carbon atoms, alkenyl of 2 to 4 carbon atoms, -(CH₂)ₚCOOH wherein p is 0, 1,-2 or 3, -NO₂, NH₂ or -NHCOCH₃, or any two of the adjacent groups are the atoms necessary to form a fused on benzene ring.

6. A composition according to Claim 1 in which the acutance dye has the formula (III) in which R₁₆ represents an alkyl group of 1 to 8 carbon atoms,
R¹⁷ represents alkyl or alkoxy of 1 to 8 carbon atoms, halogen, NO₂ or aryl,
R¹⁶ represents hydrogen, alkyl of 1 to 8 carbon atoms or alkoxy of 1 to 8 carbon atoms, and
X, Z and Z' independently represent hydrogen, NO₂, CN, halogen and perfluoroalkyl of 1 to 4 carbon atoms with the proviso that at least one of X and Z represent N0₂.

7. A light-sensitive composition as claimed in Claim 1 in which k=0, n=1, R² represents COOC₂H₅, C₆H₅, an alkyl group of 1 to 4 carbon atoms or hydrogen and Y is NO₂.

8. A light-sensitive composition as claimed in Claim 1 in which m=1, k=1, n=0, D is oxygen or sulphur, R² is COOR¹, C₆H₅, a substituted phenyl group of molecular weight less than 350, an alkyl group of 1 to 4 carbon atoms or hydrogen and Y is NO₂.

9. A light-sensitive composition as claimed in any preceding claim, in which the dye is used in an amount of from 5 x 10-⁴ to 0.1 mole per kilogram of total dry solids in the composition.

10. A compound suitable for use as an acutance dye having the general formula: wherein:
R¹ represents an alkyl group containing 1 to 12 carbon atoms,
R³, R⁴ and R⁵ are cyanine dyes compatible substituents,
D represents in which R⁷ is an alkyl group containing 1 to 4 carbon atoms,
n is 1 when k is 0 or k is 1 when n is 0,
m is 0, 1 or 2,
when m is 0 or 2:
R² represents an alkyl group of from 1 to 4 carbon atoms, a phenyl group, a substituted phenyl group of molecular weight less than 350, ―COOR¹ wherein R¹ is as defined above, C₆H₅CO- or R⁶NH.CO wherein R⁶ is a hydrogen atom or an alkyl, aryl or aralkyl group,
and when m is 1
R² represents R⁶NH.CO wherein R⁶ is as defined above, the free bonds in the methine group of the acutance dye being satisfied by hydrogen or substituents conventional in such groups in methine dyes and those free bonds when D is being satisfied by hydrogen or substituents which can be present in a cyanine dye type heterocyclic nucleus.

11. A method of preparing a compound as defined in Claim 10 which comprises reacting a compound of the general formula: wherein:
R¹, R³, R⁴, R⁵, D, k, n and m are as defined in Claim 10,
X⁸ represents an anion,
Z³ is selected from the group consisting of SR¹, in which R¹ is as defined in Claim 10, and with a compound of the formula: wherein Y and R² are as defined in Claim 10, the reaction being conducted in the presence of a polar solvent, a base catalyst and an acid binding agent.

## Revendications

1. Une composition photosensible comprenant un mélange intime d'un composé d'argent pratiquement insensible à la lumière qui, après réduction, produit un changement visible et suffisamment d'halogénure d'argent pour catalyser ladite réduction pour former un changement visible dans les zones où l'halogénure d'argent a été exposé à la lumière et lorsque le mélange est chauffé en présence d'un agent réducteur, la composition contenant un colorant-d'acutance, caractérisée en ce que le colorant d'acutance est un composé de formule générale: où R¹ représente un radical alkyle contenant 1 à 12 atomes de carbone,
R² représente un atome d'hydrogène, un radical alkyle de 1 à 4 atomes de carbone, un radical phényle, un radical phényle substitué ayant un poids moléculaire inférieur à 350, ―COOR¹ où R¹ est comme défini ci-dessus, C₆H₅CO― ou R⁶NH.CO où R⁶ représente un atome d'hydrogène ou un radical alkyle, aryle ou aralkyle,
R³, R⁴ et R⁵ représentent indépendamment un atome d'hydrogène ou un substituant qui peut être présent dans un noyau hétérocyclique de type colorant de cyanine,
D représente où R⁷ représente un radical alkyle contenant 1 à 4 atomes de carbone,
Y représente -CN ou -NO₂,
n est 1 lorsque k est 0 ou k est 1 lorsque n est 0, et
m est 0, 1 ou 2,
les liaisons libres du radical méthine du colorant d'acutance étant satisfaites par l'hydrogène ou des substituants classiques de tels radicaux des colorants de méthine et ces liaisons libres lorsque D est étant satisfaites par l'hydrogène ou des substituants qui peuvent être présents dans un noyau hétérocyclique de type colorant de cyanine.

2. Une composition selon la revendication 1, dans laquelle le colorant d'acutance est un 1-alkyl-4- j nitrométhylène-quinolane, le substituant alkyle contenant 1 à 4 atomes de carbone.

.3. Une composition selon la revendication 2, dans laquelle le colorant d'acutance répond à la formule générale (II): où R¹¹ représente un radical alkyl contenant 1 à 4 atomes de carbone, chaque R¹² représente indépendamment un atome d'hydrogène ou d'halogène, un radical alkyle ou alcoxy contenant 1 à 4 atomes de carbone, un radical alcényle contenant 2 à 4 atomes de carbone, ―(CH₂)ₚCOOH où p est 0, 1, 2 ou 3, -N0₂, -NH₂ ou NHCOCH₃, ou deux radicaux R¹² représentent ensemble les atomes de carbone nécessaires pour achever un cycle condensé sur le benzène.

4. Une composition photosensible comme revendiqué dans la revendication 3, où R¹¹ représente un radical méthyle ou éthyle, au moins un radical R¹² représente un atome d'hydrogène et chaque autre R¹² représente indépendamment un atome d'hydrogène, de chlore ou de brome ou un radical méthyle, éthyle, éthoxy ou méthoxy.

5. Une composition comme revendiqué dans la revendication 1 où R² représente: où X, Z et Z' représentent indépendamment un atome d'hydrogène ou d'halogène, NO₂, CN ou un perfluoroalkyle de 1 à 4 atomes de carbone, avec la restriction qu'au moins un de X et Z est N0₂ et R³ et R⁵ représentent indépendamment un atome d'hydrogène ou d'halogène, un alkyle ou un alcoxy de 1 à 4 atomes de carbone, un alcényle de 2 à 4 atomes de carbone, ―(CH₂)ₚCOOH où p est 0, 1, 2 ou 3, -N0₂, NH₂ ou -NHCOCH₃, ou deux quelconques des radicaux adjacents sont les atomes nécessaires pour former un cycle condensé sur le benzène.

6. Une composition selon la revendication 1, dans laquelle le colorant d'acutance répond à la formule (III): où R¹⁸ représente un radical alkyle de 1 à 8 atomes de carbone,
aryle, R¹⁷ représente un radical alkyle ou alcoxy de 1 à 8 atomes de carbone, un halogène, NO₂ ou un
R¹⁸ représente un hydrogène, un alkyle de 1 à 8 atomes de carbone ou un âlcoxy de 1 à 8 atomes de carbone, et
X, Z et Z' représentent indépendamment un hydrogène, NO₂, CN, un halogène ou un perfluoroalkyle de 1 à 4 atomes de carbone avec la restriction qu'au moins 1 de X et Z représente NO₂.

7. Une composition photosensible comme revendiqué dans la revendication 1, où k = 0, n = 1, R² représente COOC₂H₅, C₆H₅, un radical alkyle de 1 à 4 atomes de carbone ou un hydrogène et Y est NO₂.

8. Une composition photosensible comme revendiqué dans la revendication 1, où m = 1, k = 1, n = 0, D est un oxygène ou un soufre, R² est COOR¹, C₆H₅, un radical phényle substitué de poids moléculaire inférieur à 350, un radical alkyle de 1 à 4 atomes de carbone ou un hydrogène et Y est NO₂.

9. Une composition photosensible comme revendiqué dans l'une des revendications précédentes, dans laquelle le colorant est utilisé à raison de 5 x 10⁻⁴ à 0,1 mole par kilogramme de matières sèches totales dans la composition.

10. Un composé convenant à l'emploi comme colorant d'acutance répondant à la formule générale: où:
R' représente un radical alkyle contenant 1 à 12 atomes de carbone,
R³, R⁴ et R⁵ sont des substituants compatibles avec un colorant de cyanine,
D représente un constituant du groupe composé par où
R⁷ est un radical alkyle contenant 1 à 4 atomes de carbone,
n est 1 lorsque k est 0 ou k est 1 lorsque n est 0,
m est 0, 1 ou 2,
lorsque m est 0 ou 2:
R² représente un radical alkyle de 1 à 4 atomes de carbone, un radical phényle, un radical phényle substitué ayant un poids moléculaire inférieur à 350, ―COOR¹ où R¹ est comme défini ci-dessus, C₆H₅CO― ou R⁶NH.CO- où R⁶ est un constituant du groupe composé par un atome d'hydrogène ou un radical alkyle, aryle ou aralkyle,
et lorsque m est 1:
R² représente R⁶NH.CO où R⁶ est comme défini ci-dessus, les liaisons libres du radical méthine du colorant d'acutance étant satisfaites par l'hydrogène ou des substituants classiques de tels radicaux des colorants de méthine et les liaisons libres lorsque D est étant satisfaites par l'hydrogène ou des substituants qui peuvent être présents aans un noyau hétérocyclique de type colorant de cyanine.

11. Un procédé pour préparer un composé comme défini dans la revendication 10, qui comprend la réaction d'un composé de formule générale: où:
R¹, R³, R⁴, R⁵, D, k, n et m sont comme définis dans la revendication 10,
X^{e} représente un anion,
Z³ est choisi parmi le groupe constitué par SR¹, où R¹ est comme défini dans la revendication 10, et avec un composé de formule où Y et R² sont comme défini dans la revendication 10, la réaction étant effectuée en présence d'un solvant polaire, d'un catalyseur basique et d'un agent fixant les acides.

## Patentansprüche

1. Eine lichtempfindliche Masse, umfassend ein inniges Gemisch aus einer im wesentlichen lichtunempfindlichen Silberverbindung, die bei Reduktion eine sichtbare Änderung ergibt und genügend Silberhalogenid, um diese Reduktion zu katalysieren, um eine sichtbare Änderung in den Bereichen zu ergeben, in denen das Silberhalogenid belichtet wurde, und wenn das Gemisch in Gegenwart eines Reduktionsmittels erhitzt wird, wobei die Masse einen Schirmfarbstoff enthält, dadurch gekennzeichnet, daß der Schirmfarbstoff eine Verbindung der allgemeinen Formel ist: in der R¹ eine Alkylrest mit 1 bis 12 Kohlenstoffatomen darstellt,
R² ein Wasserstoffatom, einen Alkylrest mit 1 bis 4 Kohlenstoffatomen, eine Phenylgruppe, eine substituierte Phenylgruppe mit einem Molekulargewicht unter 350, -COOR', wobei R¹ wie vorstehend definiert ist, C₆H₅CO― oder R⁶NH.CO―,
wobei R⁶ eine Wasserstoffatom oder einen Alkyl-, Aryl- oder Aralkylrest bedeutet, darstellt, R³, R⁴ und R⁵ unabhängig voneinander ein Wasserstoffatom oder einen Substituenten bedeuten, der in einem heterocyclischen Kern des Cyaninfarbstofftyps enthalten sein kann, darstellt, wobei R⁷ einen Alkylrest mit 1 bis 4 Kohlenstoffatomen bedeutet,
Y -CN oder -N0₂ bedeutet,
n 1 ist, wenn k 0 ist oder k 1 ist, wenn n 0 ist, und
m 0, 1 oder 2 ist, wobei die freien Bindungen in der Methingruppe des Schirmfarbstoffs durch Wasserstoff oder bei Methinfarbstoffen in diesen Gruppen übliche Substituenten abgesättigt sind und die freien Bindungen, wenn D die Gruppe ist, durch Wasserstoff oder Substituenten abgesättigt sind, die in einem heterocyclischen Kern des Cyaninfarbstofftyps anwesend sein können.

2. Eine Masse nach Anspruch 1, in der der Schirmfarbstoff ein 1-Alkyl-4-nitromethylen-chinolan ist, wobei der Alkylsubstituent 1 bis 4 Kohlenstoffatome enthält.

3. Eine Masse nach Anspruch 2, in der der Schirmfarbstoff die allgemeine Formel (II) hat: in der R¹¹ einen Alkylrest mit 1 bis 4 Kohlenstoffatomen bedeutet, jeder Rest R¹² unabhängig ein Wasserstoff- oder Halogenatom, einen Alkyl- oder Alkoxyrest mit 1 bis 4 Kohlenstoffatomen, einen Alkenylrest mit 2 bis 4 Kohlenstoffatomen, ―(CH₂)ₚCOOH, wobei p 0, 1, 2 oder 3 ist, ―NO₂, ―NH₂ oder ―NHCOCH₃ bedeutet, oder zwei Reste R¹² zusammen die zum Vervollständigen eines ankondensierten Benzolrings erforderlichen Kohlenstoffatome darstellen.

4. Eine lichtempfindliche Masse nach Anspruch 3, in der R¹¹ eine Methyl- oder Äthylgruppe bedeutet, mindestens ein Rest R¹² ein Wasserstoffatom darstellt und alle anderen Reste R¹² unabhängig voneinander ein Wasserstoff-, Chlor- oder Bromatom oder eine Methyl-, Äthyl-, Methoxy- oder Äthoxygruppe darstellen.

5. Eine Masse nach Anspruch 1, in der R² bedeutet: in der X, Z und Z' unabhängig ein Wasserstoff- oder Halogenatom, -N0₂, -CN oder Perfluoralkyl mit 1 bis 4 Kohlenstoffatomen bedeuten, mit der Maßgabe, daß mindestens einer der Reste X und Z ―NO₂ ist und R³, R⁴ und R⁵ unabhängig ein Wasserstoff- oder Halogenatom, einen Alkyl- oder Alkoxyrest mit 1 bis 4 Kohlenstoffatomen, einen Alkenylrest mit 2 bis 4 Kohlenstoffatomen, ―(CH₂)ₚCOOH, wobei p 0, 1, 2 oder 3 ist, ―NO₂, -NH₂ oder ―NHCOCH₃ bedeuten, oder irgendwelche zwei benachbarte Reste, die zur Bildung eines ankondensierten Benzolrings notwendigen Atome sind.

6. Eine Masse nach Anspruch 1, in der der Schirmfarbstoff die Formel (III) hat: in der R¹⁶ einen Alkylrest mit 1 bis 8 Kohlenstoffatomen darstellt,
R¹⁷ einen Alkyl- oder Alkoxyrest mit 1 bis 8 Kohlenstoffatomen, ein Halogenatom, ―NO₂ oder einen Arylrest bedeutet, R¹⁸ ein Wasserstoffatom, einen Alkylrest mit 1 bis 8 Kohlenstoffatomen oder einen Alkoxyrest mit 1 bis 8 Kohlenstoffatomen darstellt und
X, Z und Z' unabhängig Wasserstoffatome, ―NO₂, ―CN, Halogenatome und Perfluoralkylreste mit 1 bis 4 Kohlenstoffatomen bedeuten, mit der Maßgabe, daß mindestens einer der Reste X und Z ―NO₂ darstellt.

7. Eine lichtempfindliche Masse gemäß Anspruch 1, in der k = 0, n = 1, R² ―COOC₂H₅, ―C₆H₅, ein Alkylrest mit 1 bis 4 Kohlenstoffatomen oder ein Wasserstoffatom und Y ―NO₂ bedeutet.

8. Eine lichtempfindliche Masse gemäß Anspruch 1, in der m = 1, k = 1, n = 0, D ein Sauerstoff-oder Schwefelatom ist, R² ―COOR¹, ―C₆H₅, eine substituierte Phenylgruppe mit einem Molekulargewicht unter 350, eine Alkylrest mit 1 bis 4 Kohlenstoffatomen oder eine Wasserstoffatom ist und Y -NO₂ ist.

9. Eine lichtempfindliche Masse nach einem oder vorangehenden Ansprüche, in welcher der Farbstoff in einer Menge von 5 x 10-⁴ bis 0,1 Mol/kg der gesamten trocknen Feststoffe in der Masse verwendet wird.

10. Eine Verbindung, die sich zur Verwendung als Schirmfarbstoff eignet und die allgemeine Formel aufweist: in der:
R' einen Alkylrest mit 1 bis 12 Kohlenstoffatomen bedeutet, R³, R⁴ und R⁵ mit Cyaninfarbstoffen verträgliche Substituenten sind,
D einen der Reste darstellt, wobei R⁷ ein Alkylrest mit 1 bis 4 Kohlenstoffatomen ist,
n 1 ist, wenn k 0 ist, oder k 1 ist, wenn n 0 ist,
m 0, 1 oder 2 ist,
wenn m 0 oder 2 ist:
R² einen Alkylrest mit 1 bis 4 Kohlenstoffatomen, eine Phenylgruppe, eine substituierte Phenylgruppe mit einem Molekulargewicht unter 350, ―COOR¹, wobei R¹ wie vorstehend definiert ist, C₆H₅CO― oder R⁶NH.CO bedeutet, wobei R⁸ ein Wasserstoffatom oder ein Alkyl-, Aryl- oder Aralkylrest ist,
und wenn m 1 ist:
R², R⁵NH.CO darstellt, wobei R⁶ wie vorstehend definiert ist, wobei die freien Bindungen in der Methingruppe des Schirmfarbstoffes durch Wasserstoffatome oder durch in solchen Gruppen in Methinfarbstoffen übliche Substituenten abgesättigt sind und jene freien Bindungen, wenn D der Rest ist, durch Wasserstoffatome oder Substituenten abgesättigt sind, die in einem heterocyclischen Kern des Cyaninfarbstofftyps anwesend sein können.

11. Ein Verfahren zur Herstellung einer Verbindung gemäß der Definition in Anspruch 10, das die Umsetzung einer Verbindung der allgemeinen Formel in der:
R¹, R³, R⁴, R⁵, D, k, n und m wie in Anspruch 10 definiert sind,
X^{e} eine Anion darstellt, und
Z³ den Rest SR¹, wobei R¹
wie in Anspruch 10 definiert ist, oder den Rest der Formel besteht: bedeutet, mit einer Verbindung der Formel umfaßt, wobei Y und R² wie in Anspruch 10 definiert sind, wobei die Umsetzung in Gegenwart eines polaren Lösungsmittels, eines basischen Katalysators und eines Säurebindemittels durchgeführt wird.
